

Dec. 31, 1963

I. S. JACOBS ET AL

3,116,254

METHOD FOR MAKING MAGNETS

Filed May 29, 1961



Inventors:  
Israel S. Jacobs;  
James S. Kouvel,

by Richard A. Speer  
Attorney

# United States Patent Office

3,116,254

Patented Dec. 31, 1963

1

3,116,254

## METHOD FOR MAKING MAGNETS

Israel S. Jacobs, Schenectady, and James S. Kouvel, Albany, N.Y., assignors to General Electric Company, a corporation of New York

Filed May 29, 1961, Ser. No. 113,410

1 Claim. (Cl. 252—62.5)

This invention relates to permanent magnets and more particularly to permanent magnets having one easy direction of magnetization and to a method for producing such magnets.

Previously known magnetic materials have been most readily magnetized along one or more axes and have been equally readily magnetizable in either direction along each axis. The magnetic properties of these materials have been measured and evaluated by several methods, perhaps the best known being the graphical representation of the hysteresis loop obtained when a magnetic field is applied to the magnetic material in such a manner as to cyclically reverse polarity. Since magnetic properties have been symmetrically reversible, both quantitatively and qualitatively with respect to the axis of magnetization, they also have at least two stable positions in a strong magnetic field.

While existing magnetic materials have generally proven acceptable for use in most situations, the increasing use of electronic and electrical apparatus in unusual environmental situations has resulted in a need for components having particular properties when subjected to such unusual conditions. For example, various parts of guidance or computer systems must be able to perform reliably at extreme temperatures. Development of these and other technological areas has resulted in recognition that a magnetic material having one easy direction of magnetization would be of value, particularly where this property could be utilized at low temperatures.

A principal object of this invention is to provide magnets having one easy direction of magnetization.

Another object of this invention is to provide a zinc or magnesium manganite permanent magnet with spinel-like crystal structure which has one easy direction of magnetization.

An additional object of this invention is to provide a process for producing magnets having one easy direction of magnetization.

Other objects and advantages of this invention will be in part obvious and in part explained by reference to the accompanying specification and drawings.

In the drawings:

FIG. 1 shows a hysteresis loop illustrating the magnetic characteristics of the usual type of permanent magnet;

FIG. 2 shows a hysteresis loop illustrating the magnetic characteristics of a magnet made according to the present invention;

FIG. 3 shows a shifted hysteresis loop of a magnet made according to the present invention of a slightly different composition from the magnet used to produce FIG. 2;

FIG. 4 shows hysteresis loops similar to the loops of FIG. 3 of materials of slightly different composition from those used in FIGS. 2 and 3; and

FIG. 5 shows hysteresis loops for the compositions used to produce FIG. 4 in which cooling in a zero magnetic field was effected.

Generally, this invention concerns permanent magnets having one easy direction of magnetization, which magnets comprise bodies having general compositions as indicated by the formulae:



where  $x$  is greater than zero and less than one.

2

The process generally comprises preparing a body of the general compositions by combining the ingredients in powder form and sintering at temperatures on the order of 1150° C. or higher in air. The sintered bodies are then quenched to room temperature, and cooled in a magnetic field to a temperature sufficiently low to create the one easy direction of magnetization within the body, this temperature normally not exceeding 30° K.

A hysteresis loop 10 characteristic of the usual type of magnet is shown in FIG. 1, in which the magnetizing field  $H$ , in oersteds, is the axis of the abscissa and the magnetization or  $M$ , in gauss, is the axis of the ordinate. As the field is increased from zero to higher values of  $H$  in what for convenience may be referred to as the positive direction, the magnetization ( $M$ ) of the material reaches a maximum value  $+M_{\max}$  for a given field. If the field  $+H$  is removed, the value of the magnetization decreases along the demagnetization curve 11 to  $M_{R1}$ . If then a field  $-H$  of reverse polarity is applied, the magnetization of the material continues to decrease along curve 11 and crosses the  $H$  axis at the value  $H_{c1}$ , the magnetization finally reaching  $-M_{\max}$  as the field is further increased in the negative direction. If the negative field is removed, the magnetization of the material correspondingly drops to  $M_{R2}$ , which is numerically equal to  $M_{R1}$ . Application of the positive field then causes the magnetization to move along the magnetization curve 12 and cross the  $H$  axis at the value  $H_{c2}$ , which is numerically equal to  $H_{c1}$ . As the positive field is increased, the magnetization of the material rises to the value  $+M_{\max}$ . The magnetization values  $M$  which were used in the present case in place of the flux density,  $B$ , to plot the hysteresis loops, are equal to the flux density ( $B$ ) minus the magnetizing field ( $H$ ), divided by  $4\pi$ , as indicated by the formula:

$$M = (B - H) / 4\pi$$

Compositions which can be used, according to the present invention, to produce magnets having one easy direction of magnetization have the general compositions indicated by the formulae:



where  $x$  is greater than zero and less than one. More specifically, compositions falling within the range of from  $\text{Zn}_{0.5}\text{Mn}_{2.75}\text{O}_4$  to  $\text{Zn}_{0.75}\text{Mn}_{2.25}\text{O}_4$  and  $\text{Mg}_{0.25}\text{Mn}_{2.75}\text{O}_4$  to  $\text{Mg}_{0.75}\text{Mn}_{2.25}\text{O}_4$  have been found to be particularly useful, although compositions outside of these ranges are also effective. These materials are single phase, as viewed by X-ray, i.e., tetragonally distorted spinel, isomorphous with the mineral Hausmannite,  $\text{Mn}_3\text{O}_4$ . The metal ions of these materials are distributed on two different kinds of crystallographic sites—tetrahedral ("A") sites and octahedral ("B") sites. In these two compounds, the B-sites are nearly completely occupied by manganese ions, while the A-sites contain mixtures of the nonmagnetic zinc or magnesium ions and the balance of the magnetic manganese ions.

The displaced character of the hysteresis loops is felt to result from an interaction between ferrimagnetic or possibly ferromagnetic regions with antiferromagnetic regions. For example, the compound  $\text{Mn}_3\text{O}_4$  is ferrimagnetic, while the compounds  $\text{ZnMn}_2\text{O}_4$  and  $\text{MgMn}_2\text{O}_4$  are most probably antiferromagnetic. On a microscopic scale, there may be composition fluctuations in the A-sites of these mixed zinc or magnesium manganites so that some parts are more like  $\text{Mn}_3\text{O}_4$  and other parts more like  $\text{ZnMn}_2\text{O}_4$  or  $\text{MgMn}_2\text{O}_4$ .

Referring to FIG. 2, curve 15 illustrates the shifted loop characteristics of a body having the general composition  $\text{Zn}_{0.5}\text{Mn}_{2.5}\text{O}_4$ . This body was produced by mix-

ing zinc oxide and manganese carbonate in the correct proportions, calcining at 1000° C. in air, grinding, pressing into pellets, firing at 1150° C. in air and quenching in air. The measurements were made on powders whose particle size ranged from about 5 microns to about 150 microns (0.15 millimeter). It is believed that the state of subdivision is not critical for the observation of the displaced hysteresis loop. The body was then cooled in a magnetic field of 5000 oersteds to a temperature of 1.7° K. It is apparent that the maximum magnetizations  $-M_{max}$  and  $+M_{max}$  are numerically the same, but the remanent magnetization values  $M_R$  are unequal as are the coercive field strengths  $H_c$ , as shown in the following Table I:

Table I

| $M_{R2}(\text{emu.})$ | $M_{R1}(\text{emu.})$ | $H_{c1}(\text{oe.})$ | $H_{c2}(\text{oe.})$ |
|-----------------------|-----------------------|----------------------|----------------------|
| 25                    | 54                    | 500                  | 100                  |

The hysteresis loop 16 of FIG. 3 of the drawings illustrates the magnetic properties of bodies produced in nearly the same manner as those used to produce FIG. 2, the composition in this case being  $Mg_{0.5}Mn_{2.5}O_4$ . The only difference is that magnesium carbonate was in place of zinc oxide. The magnetization and field values of these bodies are listed in the following Table II:

Table II

| $M_{R2}(\text{emu.})$ | $M_{R1}(\text{emu.})$ | $H_{c1}(\text{oe.})$ | $H_{c2}(\text{oe.})$ |
|-----------------------|-----------------------|----------------------|----------------------|
| 10                    | 53                    | 1,000                | 150                  |

The composition of the bodies used to obtain the curves 20 and 21 of FIG. 4 of the drawings had the compositions: (a)  $Zn_{0.25}Mn_{2.75}O_4$ ; and (b)  $Zn_{0.75}Mn_{2.25}O_4$ . In this case, the bodies were subjected to an applied magnetic field of 5000 oersteds during cooling to 1.7° K. Magnetic properties of these materials are listed in Table III:

Table III

| Sample   | Field Applied (oe.) | $M_{R1}(\text{emu.})$ | $M_{R2}(\text{emu.})$ | $H_{c1}(\text{oe.})$ | $H_{c2}(\text{oe.})$ |
|----------|---------------------|-----------------------|-----------------------|----------------------|----------------------|
| (a)----- | 5,000               | 110                   | 0                     | 700                  | 0                    |
| (b)----- | 5,000               | 2.5                   | 0                     | 400                  | 0                    |

Data similar to that contained in Table III was obtained from samples of the same compositions, specifically (a)  $Zn_{0.25}Mn_{2.75}O_4$  and (b)  $Zn_{0.75}Mn_{2.25}O_4$ . In this instance, cooling to 1.7° K was effected without the ap-

lication of a magnetic field. The properties of these materials are shown graphically as in curves 25 and 26 of FIG. 5 of the drawings and listed in the following Table IV:

Table IV

| Sample      | Field Applied (oe.) | $M_{R1}(\text{emu.})$ | $M_{R2}(\text{emu.})$ | $H_{c1}(\text{oe.})$ | $H_{c2}(\text{oe.})$ |
|-------------|---------------------|-----------------------|-----------------------|----------------------|----------------------|
| 10 (a)----- | 0                   | 30                    | 30                    | 300                  | 300                  |
| 10 (b)----- | 0                   | 2                     | 2                     | 0.1                  | 0.1                  |

The properties listed in Table IV clearly show that the magnetic properties are isotropic when no magnetic field is applied during cooling.

It is felt that the present magnets as processed acquire their unique behavior by virtue of the ferrimagnetic (or ferromagnetic) and antiferromagnetic regions present within the body. The coupling effect between these regions results in the one easy direction of magnetization. Therefore, during cooling of the body from room temperature, it is essential, as shown by FIGS. 4 and 5 of the drawings, that it be subjected to a magnetic field, one on the order of 5000 oersteds normally being sufficient to properly orient the antiferromagnetic as well as the ferrimagnetic or ferromagnetic moments. Although the magnetic field need only be applied from just above the temperature at which the shifted loop effect begins, generally 30° K. or less, as a matter of expedience, it is normally easier to apply the field continuously during the entire cooling treatment.

Although the present invention has been described in connection with preferred embodiments, it is to be understood that modifications and variations may be resorted to without departing from the spirit and scope of the invention, as those skilled in the art will readily understand. Such modifications and variations are considered to be within the purview and scope of the invention and the appended claim.

What we claim as new and desired to secure by Letters Patent of the United States is:

In the process of producing a magnet having one easy direction of magnetization, the steps comprising preparing a sintered body having a composition according to the formula selected from the group consisting of  $Zn_{0.25-0.75}Mn_{2.25-2.75}O_4$  and  $Mg_{0.25-0.75}Mn_{2.25-2.75}O_4$ , quenching the body from sintering temperature down to room temperature, cooling the body to a temperature of about 30° K. or less and subjecting the body to a magnetic field during cooling to develop the one easy direction of magnetization within the body.

#### References Cited in the file of this patent

Jacobs: J. of Applied Physics, Supp. to vol. 30, No. 4, April 1959, pages 301S and 302S.